

March 4, 1924.

1,485,505

G. HOLST ET AL  
PROCESS FOR INTRODUCING ALKALI OR EARTH ALKALI METALS IN DISCHARGING  
TUBES AND THE LIKE  
Filed Oct. 26. 1920

Fig:1.



Fig:2.



Fig:4.



Fig:3.



Inventors:  
Gilles Holst and  
Eko Oosterhuis,  
By Attorneys,  
Drasen, Dunk & Meyer

## UNITED STATES PATENT OFFICE.

GILLES HOLST AND EKKO OOSTERHUIS, OF EINDHOVEN, NETHERLANDS, ASSIGNEES  
TO NAAMLOOZE VENNOOTSCHAP PHILIP'S GLOEILAMPEN-FABRIEKEN, OF EINDHOVEN, NETHERLANDS.

## PROCESS FOR INTRODUCING ALKALI OR EARTH-ALKALI METALS IN DISCHARGING TUBES AND THE LIKE.

Application filed October 28, 1920. Serial No. 419,659.

*To all whom it may concern:*

Be it known that we, GILLES HOLST and EKKO OOSTERHUIS, both subjects of the Queen of the Netherlands, residing at Eindhoven, in the Province of North Brabant, in the Kingdom of the Netherlands, have invented certain new and useful Improvements in a Process for Introducing Alkali or Earth-Alkali Metals in Discharging Tubes and the like (for which I have filed an application in Kingdom of the Netherlands on September 23, 1919, Serial No. 12966, Ned.), of which the following is a specification.

This invention relates to vacuum or discharge tubes (incandescent lamps, X-ray tubes, audions, rectifiers, etc.), being vessels used electrically and exhausted of air to form a vacuum, or filled with suitable gases at or below atmospheric pressure. For want of a suitable generic term such devices will be herein referred to as "evacuated container electrical apparatus," or evacuated containers.

It is known, that substances such as calcium, barium, strontium, potassium, sodium, etc., in gaseous condition combine with all gases except the noble gases, whereby compositions are formed which have very low vapor pressures. This action is greatly accelerated by electrical discharges.

In such evacuated containers all gases present or set free, except the noble gases, will quickly disappear in the presence of said metals, so that a high vacuum or a very pure noble gas filling is obtained.

It has already been proposed to use heated earth-alkali metals for the absorbing of gas residues (German Patent 179526).

It has also been proposed in discharging tubes to use electrodes composed of an alkali metal or an alkali metal alloy (French Patent 451846, British Patent 29104/1912). Though in this case the alkali metal also absorbs eventual gas residues, yet the principal function of the alkali metal is to coat in the discharge. According to these patents the alkali metal is used for decreasing the tension of discharge. Therefore the cathode must consist wholly or for a large part of an alkali metal, and the decrease of the discharge tension would cease when all

the alkali metal of the electrodes has been volatilized to the colder parts of the tube.

The present invention provides a method of introducing alkali or earth alkali metals in such evacuated containers, without composing the electrodes of these metals and without these metals being vehicles of discharge.

The invention consists in introducing alkali or earth alkali-metals in such evacuated containers in order to remove the last gas residues or to purify noble gases; it is characterized by this, that in the tube or the like an alloy of an alkali or earth alkali metal (such as potassium or calcium) with a noble metal of low vapor pressure (such as tin) is applied at a place where a sufficiently high temperature is obtained to vaporize the alkali- or earth alkali metal, whereas the other component of the alloy does not evaporate to a perceptible extent.

As the only object of the alkali or earth alkali metals is to absorb small quantities of gases present or set free, only very small quantities of these metals are necessary, because they may be used up when no more gases are set free.

When applying the process according to the invention one should take care that the alloy is not put in places where the vapor of the alkali or earth alkali metal might acquire such a tension, that it would take part in the discharge.

The following are examples of suitable alloys for the practice of the present invention:

1. Tin, 96%, calcium, 4%.
2. Tin, 95.7%, potassium, 4.3%.

The use of said alloys has several advantages. In the first place the active metal is protected by the nobler metal against oxidation, moisture and other influences. At the same time the handling of these active metals is thereby without any danger.

A further advantage is, that the alloy may be put into the container in a very simple way. If one uses for instance a tin alloy this may be used as a solder upon one of the metal parts in the tube.

The accompanying drawing shows one way in which the invention may be applied, Fig. 1 being an elevation of a dis-

charge tube; Fig. 2 an elevation of the cathode part thereof; Fig. 3 an elevation of the anode; and Fig. 4 an elevation of the anode part.

5 In these drawings *a* is the anode which consists of a cylindrical plate upon which the alloy is applied on a small area on the outer side; the cathode wires are melted in the glass at *b* and the anode wires at *c*. The 10 illustrated construction is given merely as an example, the invention not being directed to any particular construction of the discharge tube or other analogous structure.

What we claim is:

15 1. Evacuated container electrical apparatus, in which an alloy of an alkali- or earth alkali-metal with a nobler metal of low vapor pressure is applied at a place where a sufficiently high temperature is obtained to

vaporize the alkali or earth-alkali metal, 20 while the other component of the alloy does not evaporate perceptibly and the vapor of the alkali or earth alkali metal does not coact in the conduction of the current.

2. Evacuated container electrical apparatus, in which a tin-calcium alloy is applied at a place where a sufficiently high temperature is obtained to vaporize the calcium 25 while the tin does not evaporate perceptibly and the calcium-vapor does not coact in the conduction of the current.

In testimony whereof we have hereunto set our signatures in the presence of a witness.

GILLES HOLST.  
EKKO OOSTERHUIS.

Witness:  
AMAN NAGTEGRAAF.